

**1**

3,515,544

**HAFNIUM ALLOYS**

Peter Harlow Morton, Solihull, and Peter Vincent McDonald Clark, Birmingham, England, assignors to Imperial Metal Industries (Kynoch) Limited, Witton, Birmingham, England, a corporation of Great Britain  
No Drawing. Filed Nov. 28, 1966, Ser. No. 597,206  
Claims priority, application Great Britain, Dec. 2, 1965,

51,234/65

Int. Cl. C22c 31/00

U.S. Cl. 75—134

9 Claims

**ABSTRACT OF THE DISCLOSURE**

Hafnium base alloys of improved tensile strength and suitable for nuclear reactor control rods consist of, by weight, 0.1–5% in total amount of one or more of the beta-stabilising elements niobium, chromium, molybdenum, nickel and iron, up to 0.5% silicon, up to 2% in total amount of at least one of the alpha stabilising elements tin and aluminum with the total alpha and beta stabilisers not exceeding 5%, balance hafnium and impurities.

This invention relates to hafnium alloys.

Hafnium is used for control rods in nuclear reactors because of its high neutron absorption coefficient. Its tensile strength is not great (about 25 tons/sq. in.) but it is very ductile and has good corrosion resistance.

We have found that the tensile strength can be improved by certain alloying additions without significant deterioration of corrosion resistance, nuclear properties or ductility.

According to the present invention, a hafnium-base alloy consists, by weight of 0.1–5% in total amount of one or more of the beta-stabilising elements niobium, chromium, molybdenum, nickel and iron, 0–0.5% silicon and optionally, 0–2% in total amount of one or both of the alpha stabilising elements, tin and aluminum, the total amount of alpha and beta stabilisers not exceeding 5%, balance hafnium and impurities.

The impurities include zirconium in amounts up to about 4%, this unusually high impurity level being due to the common mineralogical source of hafnium and zirconium. Such a quantity of zirconium does not adversely affect the properties and hafnium having a high zirconium content is cheaper than purer grades.

The effect of the beta stabilising elements is to strengthen hafnium; the alpha stabilising elements, whilst having little effect on strength when added alone, generally improve the properties of the beta stabilised alloy.

The addition of small percentages of beta stabilisers produces marked improvements in tensile strength and proof stress whilst good ductility is retained. There is a difference in the effectiveness of individual beta stabilisers in raising the tensile properties and molybdenum is particularly effective in this respect. Where more than one beta stabiliser is present, certain combinations are more effective than others, for example, chromium and silicon are more effective than niobium and molybdenum which, in turn, are better than chromium and molybdenum.

The effect of alpha stabilisers on tensile properties is a further small increase in tensile strength and proof

**2**

stress with some loss of ductility. Certain groups of alpha and beta stabilisers are more effective than others as can be seen from the tables appended hereto and the more complex alloys, in general, have the greatest strength though the ductility and proof stress vary with the combination of elements. The best alloys have twice the tensile strength and proof stress of hafnium with half the ductility.

From the results of tests recorded in the tables, preferred ranges of composition are as follows:

15 0.15–1.25% Cr  
0.1–0.40% Mo  
0.5–2.0% Nb  
0.15–0.75% Fe  
0.15–0.5% Ni  
0.6–0.8% Cr and 0.8–1.2% Si  
0.6–0.8% Cr and 0.75–2.0% Sn

20 Corrosion resistance depends upon the alloying elements added and the amount present. Chromium and nickel have least effect whilst molybdenum has a marked effect on the surface appearance. Certain of the more complex alloys have better corrosion resistance than certain binary alloy compositions, but the difference between pure hafnium and alloys having the least corrosion resistance to high temperature pressurised steam is one of small degree.

25 The corrosion resistance of the alloys of the invention was determined by exposing cleaned bright samples to steam at a pressure of 100 atmospheres and at a temperature of 400° C. for 72 hours. The corrosion behaviour of the alloys was compared by the appearance of the surface of the samples in accordance with the following classification.

- 30 35 (A) Glossy, bright, thin, adherent film (including interference films).  
(B) Glossy, bright, thick, adherent film.  
(C) Mottled appearance with dull patches or streaks which are usually powdery.  
(D) Dull but adherent uniform film.

40 45 It is important that the film should be adherent with no tendency to powder or to flake off. In the above classification, class (A) has the best corrosion resistance.

Because the alloying elements are present in small amounts, the nuclear properties are not significantly affected.

50 55 The tensile properties and corrosion resistance of a number of alloys in accordance with the invention are shown by way of example in Tables I and II in comparison with pure hafnium. The tensile tests were carried out on rod and in the tables the abbreviation  $4\sqrt{A}$ , used in connection with the elongation values, refers to the gauge length of test pieces, that is, a gauge length equal to four times the square root of the area of the cross-section of the test piece. The corrosion resistance was determined in accordance with the above classification.

60 In Table III are shown examples of the improvement in the strength of sheet produced from alloys in accordance with the invention compared with commercially pure hafnium sheet. Values for specimens cut in the longitudinal and transverse directions of the sheet are given.

It will be observed that the alloy B(L), Hf-1.1Sn-0.6Cr is heat-treatable to produce marked increases in tensile strength and proof stress whilst the ductility remains at a high level.

TABLE I

Hafnium rich alloys containing 1-5% of one or more of the beta stabilising elements: Cr, Mo, Nb, Ni, Fe or 0-0.5% Si

| Alloy             | Nominal composition | Corrosion resistance | 0.2% P.S., t.s.i. | U.T.S., t.s.i. | Elongation, percent on $4\sqrt{A}$ |
|-------------------|---------------------|----------------------|-------------------|----------------|------------------------------------|
| Unalloyed hafnium |                     |                      | 15.6              | 25.3           | 26                                 |
| Cr2               | 0.15% Cr            | A                    | 18.3              | 28.1           | 33                                 |
| Cr3               | 0.5% Cr             | A                    | 23.7              | 32.2           | 29                                 |
| Cr4               | 0.75% Cr            | A                    | 25.5              | 27.1           | 20                                 |
| Cr5               | 1.2% Cr             | A                    | 24.8              | 39.0           | 16                                 |
| Mo1               | 0.1% Mo             | A                    | 15.3              | 29.2           | 30                                 |
| Mo2               | 0.35% Mo            | A                    | 23.1              | 34.6           | 18                                 |
| Mo6               | 0.5% Mo             | C                    | 18.6              | 35.4           | 26                                 |
| Mo3               | 0.75% Mo            | C                    | 39.2              | 42.7           | 23                                 |
| Nb1               | 0.5% Nb             | A                    | 17.1              | 30.6           | 26                                 |
| Nb9               | 1.8% Nb             | A                    | 24.0              | 34.7           | 13                                 |
| Nb7               | 2.33% Nb            | C                    | 31.9              | 41.5           | 25                                 |
| Nb3               | 5.0% Nb             | D                    | 46                | 48.5           | 20                                 |
| T11               | 0.5Nb-0.35Mo        | C                    | 32.3              | 44.3           | 18                                 |
| T12               | 1.5Nb-0.35Mo        | C                    | 38.3              | 45.2           | 27                                 |
| T15               | 0.75Cr-0.5Mo        | C                    | 25.2              | 39.5           | 13                                 |
| T18               | 0.75Cr-0.15Si       | A                    | 32.9              | 50.0           | 5                                  |
| Fe1               | 0.15% Fe            | A                    | 15.8              | 30.6           | 17                                 |
| Fe3               | 0.75% Fe            | A                    | 21.2              | 35.4           | 10                                 |
| Ni3               | 0.15% Ni            | A                    | 22.6              | 32.2           | 26                                 |
| Ni4               | 0.25% Ni            | A                    | 16.1              | 33.1           | 20                                 |
| Ni5               | 0.5% Ni             | A                    | 15.9              | 32.1           | 25                                 |

TABLE II

Hafnium-rich alloys containing 1-5% of one or more of the beta stabilising elements: Cr, Mo, Nb, Ni, Fe, 0-0.5% Si, together with 0-2% of one or more of the alpha stabilising elements, Sn, Al

| Alloy   | Nominal composition              | Corro-<br>sion re-<br>sistance | 0.2% P.<br>S., t.s.i. | U.T.S.,<br>t.s.i. | Elonga-<br>tion, per<br>cent on<br>$4\sqrt{A}$ |
|---------|----------------------------------|--------------------------------|-----------------------|-------------------|------------------------------------------------|
| T10     | 2.3Nb-0.25Al                     | C                              | 34.7                  | 45.5              | 23                                             |
| T9      | 2.3Nb-0.8Sn                      | C                              | 35.0                  | 47.3              | 40                                             |
| T8      | 0.75Mo-0.8Sn                     | C                              | 30.4                  | 43.9              | 18                                             |
| T24     | 0.75Mo-0.3Al                     | C                              | 36.5                  | 48.0              | 5                                              |
| T13     | 0.75Cr-0.5Al                     | B                              | Not determined        |                   |                                                |
| T16     | 0.75Cr-0.8Sn                     | A                              | 28.4                  | 38.1              | 8                                              |
| T17     | 0.75Cr-2.0Sn                     | A                              | 28.3                  | 42.5              | 11                                             |
| Alloy B | 0.8Cr-1.5Sn                      | A                              | Not determined        |                   |                                                |
| Q3      | 0.75Cr-0.8Sn-0.01Si              | C                              | 40.8                  | 49.8              | 6                                              |
| Q4      | 0.75Mo-0.8Sn-0.2Si               | C                              | 39.1                  | 51.5              | 15                                             |
| C1      | {0.75Sn-0.05Cr<br>0.06Fe-0.02Ni} | A                              | 28.3                  | 46.6              | 10                                             |

TABLE III.—TENSILE PROPERTIES OF STRIP

| Alloy                                                             | Analysed composition | Direction of specimen | 0.2% P.S., t.s.i. | U.T.S., t.s.i. | Percent Elongation on 1 in. |
|-------------------------------------------------------------------|----------------------|-----------------------|-------------------|----------------|-----------------------------|
| 5 A(R)                                                            | 0.55 Cr              | Long...               | 16.1              | 33             | 30                          |
|                                                                   |                      | Trans...              | 24.1              | 32.9           | 32                          |
| B(L)                                                              | 1.1 Sn-0.6 Cr        | Long...               | 16.6              | 30.9           | 40                          |
|                                                                   |                      | Trans...              | 18.2              | 30.3           | 44                          |
| B(L) cold rolled and heat treated 1 hr. 750° C. and 1 hr. 850° C. | 1.1 Sn-0.6 Cr        | Trans...              | 25.3              | 34.0           | 33                          |
| Pure hafnium                                                      |                      | Long...               | 9.4               | 25.3           | 35                          |
|                                                                   |                      | Trans...              | 14.59             | 24.89          | 41                          |

We claim:

1. A hafnium-base alloy consisting by weight of 0.1%-5% in total amount of at least one beta-stabilising element selected from the group consisting of niobium, chromium, molybdenum, nickel and iron; up to 0.5% silicon, and up to 2% in total amount of at least one alpha stabilising element selected from the group consisting of tin and aluminium, the total amount of alpha and beta stabilisers not exceeding 5%; balance hafnium and impurities.
2. A hafnium-base alloy according to claim 1 containing 0.15-1.25% chromium.
3. A hafnium-base alloy according to claim 1 containing 0.1-0.40% molybdenum.
4. A hafnium-base alloy according to claim 1 containing 0.5-2.0% niobium.
5. A hafnium-base alloy according to claim 1 containing 0.15%-0.75% iron.
6. A hafnium-base alloy according to claim 1 containing 0.15-0.5% nickel.
7. A hafnium-base alloy according to claim 1 containing 0.6-0.8% chromium and 0.8-1.2% silicon.
8. A hafnium-base alloy according to claim 1 containing 0.6-0.8% chromium and 0.75-2.0% tin.
9. A hafnium-base alloy according to claim 1 consisting of 0.75% tin, 0.05% chromium, 0.06% iron and 0.02% nickel, balance hafnium apart from impurities.

#### References Cited

#### UNITED STATES PATENTS

- 45 2,234,969 3/1941 Hensel et al. ----- 75—134  
2,810,640 10/1957 Bolkcom et al. ----- 75—134

RICHARD O. DEAN, Primary Examiner